

E. J. KEITH,  
METHOD OF PROTECTING BEARING SURFACES.  
APPLICATION FILED JUNE 3, 1918.

**1,318,766.**

Patented Oct. 14, 1919.



WITNESS.

*Charles A. Becket*

BY

INVENTOR.

*E. J. Keith*  
*Kingman Cook*

HIS ATTORNEYS.

# UNITED STATES PATENT OFFICE.

EPHRAIM J. KEITH, OF SIKESTON, MISSOURI, ASSIGNOR OF FORTY-FIVE ONE-HUNDREDTHS TO MATTHEW S. MURRAY, OF SIKESTON, MISSOURI, AND TEN ONE-HUNDREDTHS TO JAMES A. FINCH, OF NEW MADRID, MISSOURI.

## METHOD OF PROTECTING BEARING-SURFACES.

1,318,766.

Patented Oct. 14, 1919.

Application filed June 3, 1918. Serial No. 238,005.

Specification of Letters Patent.

To all whom it may concern:

Be it known that I, EPHRAIM J. KEITH, a citizen of the United States of America, a resident of Sikeston, in the county of Scott, 5 State of Missouri, have invented certain new and useful Improvements in Methods of Protecting Bearing-Surfaces, of which the following is a full, clear, and exact description, reference being had to the accompanying drawings, forming a part of this specification.

My invention relates to a means for protecting bearing surfaces, such as wire ropes or cables, and the sheaves or pulleys on 15 which they operate, gears, sprockets and chains or other objects subjected to frictional wear, and to a method of applying such means to the objects to be protected. The means to which my invention relates and 20 the method of applying it are intended primarily for use in protecting wire ropes and the sheaves on which they operate, and in the description given herein I will confine myself to such use of the means and method 25 without in any way limiting myself in so doing.

The accompanying drawing is a section through a fragment of a sheave and a section of wire rope, with my protecting means applied to both elements as an example 30 of the utility of my invention.

In the drawing A designates a wire rope and B designates a sheave serving as a support and guide for the wire rope, said sheave 35 having the usual peripheral groove.

It is a matter of general knowledge among users of wire rope that the strands of such a rope create great wear upon the sheaves they operate upon, in time creating grooves 40 in the peripheries of the sheaves with ridges between them, which result in rapid wear of the ropes and the sheaves. This is true, notwithstanding the application of the lubricants to the ropes and sheaves which form 45 only a thin film of friction reducing medium and do not in any very material measure lessen the wear and destruction of the contacting parts. By my improvement I so coat the contact surfaces of the ropes 50 and sheaves as to separate them from each other and avoid the wear of one metal part against the other, and as a consequence eliminate the possibility of the wire rope cutting into the sheave and the resultant in-

jury to the wire rope, due to such cutting in 55 operation.

The medium I use to coat the contact surfaces of the wire rope and sheave is a self-solidifying substance, preferably asphalt, which may be used either alone or impregnated with a suitable binder of fibrous material, for example, asbestos or mineral wool.

In preparing asphalt for use as a protective coating for coöperating mechanical 65 elements I take asphalt which has been freed of volatile oils and heat it to a sufficient degree of temperature to render it fluid or semi-fluid, and while the asphalt is in such condition apply it to the elements it is to 70 protect. The asphalt adheres to such elements and, upon cooling, becomes solidified so that it remains firmly attached thereto, forming mats thereon or therearound. In practical use I have found that the most 75 advantageous way of applying the coating to a wire rope and a sheave on which it operates is by pouring the asphalt while in a fluid or semi-fluid condition onto the rope and sheave while they are in motion, the 80 asphalt congealing when it touches the elements it is to protect and then becoming built up thereon to form solid coverings, which serve to maintain the elements out 85 of contact with each other.

In the example illustrated 1 designates the covering applied to the wire rope and 2 the covering applied to the sheave. In following the procedure I have described, the asphalt during congealment is built up into 90 a substantially uniform mat at the periphery of the sheave, between it and the wire rope, and a substantially uniform mat of the asphalt is also formed on the wire rope, any excess of asphalt employed for the coatings 95 being expressed outwardly onto the edges of the flanges of the sheave, as shown.

I have hereinbefore made mention of the inclusion of binding or filling material in the asphalt. Such material may or may not be 100 used in all instances, but is preferably used where heavy duty cables are employed and in the use of which the protecting coatings would be subjected to severe pressure and strain.

I claim:

1. The method of applying protective coatings to the bearing surfaces of two co-

operating mechanical elements, which consists in placing a heated self-solidifying substance in contact with said elements while they are in motion, causing said substance to be introduced between said elements while congealing thereon.

2. The method of applying protective coatings to the bearing surfaces of wire ropes and sheaves, which consists in placing a heated congealable substance in contact with one of said elements, and moving said elements during congelation of said substance

to cause the substance to be introduced between the elements while congealing thereon.

3. The method of applying protective 15 coatings to wire ropes and sheaves, which consists in pouring a fluid or semifluid congealable substance onto a wire rope and sheave while the wire rope is moving on the sheave, and permitting said substance to 20 congeal on said members.

In testimony that I claim the foregoing I hereunto affix my signature.

EPHRAIM J. KEITH.

**Copies of this patent may be obtained for five cents each, by addressing the "Commissioner of Patents, Washington, D. C."**